

## UNITED STATES PATENT OFFICE

2,572,903

PHOTOGRAPHIC DEVELOPER CONTAINING  
THALLIUM SALTSJames E. Bates, Binghamton, N. Y., assignor to  
General Aniline & Film Corporation, New York,  
N. Y., a corporation of DelawareNo Drawing. Application October 30, 1947,  
Serial No. 783,224

3 Claims. (Cl. 95—88)

1

This invention relates to the development of photographic emulsions of the reversible color type on films and other transparent materials for the production of positive color transparencies and the development of such emulsions on paper and other printing material for the production of color positive prints from the said transparencies by the color reversal process and, in particular, it relates to improvements in the developing solutions and in the process of developing the color reversal emulsions.

This application is a continuation-in-part of my application Serial No. 541,649 filed June 22, 1944, for "Photographic Emulsion Development" (now abandoned).

In the commercial practice of developing photographic emulsions where a large quantity of the photographic film is to be developed, it is desirable that all the film be subjected to the developing solution for the same length of time. However, this is rendered difficult because after a number of photographic films have been developed in a given solution, there is a gradual change in tone of the developed film and a loss of developing energy of the solution. Consequently, unless the time of development is increased, it is not possible to produce a satisfactory density and contrast. Heretofore it was believed that loss in developing energy of the solution, and consequent increase in time of development, was due to depletion of the developing agent and it has been proposed to maintain a relatively uniform development time by replenishing the developer solution. Such replenishment has not been satisfactory as there occurs a relatively large shift in development energy of the solution for each portion of film developed for which adequate compensation can be made only by increasing the time of development.

The contrast obtained with a given exposure of film is dependent to a large extent upon the time of development, but a maximum contrast is limited by the maximum gradation of the curve representing density plotted against the logarithm of the time of development. For many purposes a high contrast is desirable, as in the case of multilayer color film to be developed by the reversal process. In the development of this type of film, it is highly desirable to obtain a high contrast while at the same time maintaining the time of development as small as possible. It is, therefore, an object of this invention to improve the developing solutions employed in the development of photographic reversible type multicolor emulsions on films, plates, papers and the like.

2

The developing process for multicolor reversible emulsions consists of six essential steps with washes and rinses interposed where necessary. After exposure of such an emulsion, it is developed in a metal-hydroquinone developer. This develops to metallic silver the three tri-color separation images recorded in the emulsion layers of a tri-pack multilayer color material. No color is formed during this development, which is designated as the first development, since color can only be formed when the film is developed in the proper color forming developer. After this first development, the film is rinsed, then short-stopped in an acetic acid short-stop to arrest development. After short-stopping, the film is washed and re-exposed. During this re-exposure or second exposure, all silver halides in the film which were not previously exposed in the camera and which did not develop in the first developer now become exposed and are ready for development in the color forming developer. These silver halides make up the positive image. In the color forming developer, these silver halides are reduced to metallic silver by the reaction of the developer. Simultaneously with the reduction of the silver halides to metallic silver, reaction products which generally occur in developing are produced. In a normal black and white film these reaction products diffuse through the gelatin and are finally washed out in the developer and subsequent baths. However, in the color film these reaction products combine with the color formers originally placed in the film and produce dye in proportion to the amount of silver halides which were reduced. Thus, as the three positive images in the film develop to metallic silver three separate dye images are formed in situ with the silver images. No color is formed around the negative image because this image is already in the reduced or metallic silver state as a consequence of the first development and no further reduction can take place.

It has been determined that the addition of soluble thallium salts, such as thallous and thallic nitrate, thallous and thallic sulfate, and thallous hydroxide, to the first developer for a reversal multilayer color film or paper emulsion materially improves the developing characteristics and prolongs the life of the developer. When unusually high emulsion speeds and increased contrasts are obtained, for example, when 50 mg. of thallium nitrate are added to a first developer of the metol-hydroquinone type and the resulting developer is used to develop a reversible color printing material exposed in a camera using a Weston speed rating of 12, adequately exposed pictures will be obtained when

## 3

first developed only 8 minutes. In the absence of the thallium compound, the same developer requires three times as much exposure and a first development time of 15 minutes to secure a comparable picture. When the thallium compound is omitted from the developer, it is necessary to extend the development time to 20 minutes in order to secure an emulsion speed of 12 which is secured by only 8 minutes development with the thallium compound present. When the first development is thus extended in order to secure this additional speed, the color balance is altered radically because of the uneven degree of development of the various layers of the color film. When a thallium compound is used, the layers develop evenly and no disturbing unbalance results. The use of thallium compounds in the first development, therefore, permits higher emulsion speed and at the same time allows maintenance of better color balance and better contrast than could be obtained by any length of developing time without the thallium compound in the developer.

The action of the thallium compounds on the first developer for reversal color film or printing material emulsions is such that it will effect the revivification of exhausted developer solutions. In applying the invention to the revivifying of developer solutions, a soluble thallium salt is intermittently added in small increments during the development process. The required amount of the soluble thallium salt may be introduced intermittently after a predetermined quantity of the film has passed through the developing solution or, where the film is developed continuously, the soluble thallium salt may be added continuously until the developer is substantially exhausted. If desired, the developer and other ingredients of the developing solution may also be replenished by addition of suitable quantities of developer, preservative and alkali, along with suitable quantities of the soluble thallium salt to maintain the desired proportions. In this method of replenishing developer solutions, a relatively small quantity of the soluble thallium salt is used, preferred amounts being about 0.001 to 0.005 gram per square foot of emulsion developed, depending upon the degree of exhaustion of the developer. The salt is added to the solution after partial exhaustion.

In order to obtain the maximum effect on contrasts, rate of development and emulsion speed, the soluble thallium salt is added to the fresh developer solution before commencing to develop emulsions therein, a quantity in the order of about 0.01 to 0.1 gram per liter of developer solution being employed. A metol-hydroquinone developer of the type used for the first development of a reversal multicolor film emulsion which has been so treated will develop more film than a similar developer which has not been treated by the addition of such quantities of soluble thallium salts, and when used as the first developer for a reversal color film emulsion or a reversal color printing paper emulsion will develop such emulsions in approximately half the time and produce higher contrasts than in the case of a developer which has not been treated with the thallium compound.

The following examples will serve to further illustrate this invention and the best manner of carrying it out, it being understood that the materials and proportions therein recited are given by way of illustration and not intended

## 4

as limitations. Unless otherwise specified, the parts are by weight.

## Example I

Multilayer color film of the type containing color formers in situ in the color sensitive layers, such as that which is currently on the market and known as Ansco Color Film (reg. T. M.), is normally processed by the following procedure:

1. First developed 12' at 68 F. in the following solution:

|                    | Grams |
|--------------------|-------|
| Metol              | 3     |
| Sodium sulfite     | 50    |
| Hydroquinone       | 6     |
| Sodium carbonate   | 40    |
| Sodium thiocyanate | 2     |
| Potassium bromide  | 2     |
| Water to make 1 l. |       |

2. Rinsed 1' in running water.

3. Hardened 5' in a 3% solution of potassium chrome alum.

4. 2nd exposed to light of photoflood lamp for 3'.

5. Color developed 18' in the following solution:

|                             | Grams |
|-----------------------------|-------|
| P-amino diethyl aniline HCl | 4.0   |
| Sodium bisulfite            | 1.0   |
| Sodium carbonate            | 67.5  |
| Potassium bromide           | 2.5   |
| Water to make 1 l.          |       |

6. Short stopped—2' in

|                    | cc | Grams |
|--------------------|----|-------|
| Acetic acid        | 10 |       |
| Sodium acetate     | 20 |       |
| Water to make 1 l. |    |       |

7. Hardened 5' in a 3% potassium chrome alum solution.

8. Washed 5'.

9. Bleached 10' in

|                          | Grams |
|--------------------------|-------|
| Potassium ferricyanide   | 60    |
| Potassium bromide        | 15    |
| Dibasic sodium phosphate | 13    |
| Sodium bisulfite         | 6     |
| Water to make 1 l.       |       |

10. Washed 5'.

11. Fixed 5' in 20% hypo solution.

12. Washed 10' and dried.

10 sheets of Ansco Color Film 8 x 10" size were developed individually and successively in 1 liter of the above first developer then subsequently short stopped. After all 10 sheets were processed in the first developer they were simultaneously given the color development and other steps to complete the reversal procedure. It was found that the 10th sheet processed in the first developer showed a speed only 40% that of the first sheet processed in the first developer. To the thus partially exhausted first developer solution was added .010 g. thallous nitrate and an additional sheet was given first development and the subsequent steps to complete the reversal process. The sheet processed after the thallous nitrate addition to the first developer showed that the speed of the film had been restored to within 20% of the original speed. Furthermore, the color of the film developed in this solution was not impaired.

## Example II

One liter of the first developer prepared as described in Example I was used for developing

## 5

25—8 x 10" exposed multilayer color film batches of 5 sheets at a time. The developer exhausted progressively and produced progressively lower emulsion speeds in the film and when all had been developed, the film showed only about one-quarter the original emulsion speed. In a similar solution the same quantity of film was processed in the same stages but the developer solution was replenished by the addition of 80 cc. of the following replenished solution after each development of 5 sheets of film:

|                    | Grams |
|--------------------|-------|
| Metol              | 4     |
| Sodium sulfite     | 50    |
| Hydroquinone       | 8     |
| Sodium carbonate   | 40    |
| Sodium thiocyanate | 5     |
| Water, 1 l.        |       |

With replenishment in this manner the emulsion speed obtained with the 25th sheet was reduced to one-half the original value which was nearly twice the speed of no replenishment at all. A third developer solution was then similarly exhausted and replenished with the same replenisher solution but to which had been added .08 gram per liter of thallous nitrate. The film processed in first developer replenished with the thallium containing replenisher showed no loss in emulsion speed after developing the 25 exposed multilayer color films.

## Example III

Multilayer color film of the reversal type was processed according to the procedure in Example I except that the first developer solution contained 0.100 gram of thallium hydroxide per liter. This film showed an emulsion speed of about 24 Weston and a gamma of about 3 to 4. Development of a similar film in a similar first developer solution having no added thallous hydroxide showed an emulsion speed of about 8 Weston and a gamma of about 1 to 2.

## Example IV

It is often desirable to obtain a color print directly from a camera exposure instead of first making a color transparency original and then making a print from the original on another multilayer reversible color print material such as Ansco Color Printon (reg. T. M.). The pictures can be made directly on the Ansco Color Printon, but the use of this as a camera material is limited because of the low emulsion speed. Attempts have been made to increase the emulsion speed to the usable level by employing greatly extended first development times. By using a development time of 20 to 24 minutes at 68 F., barely passable emulsion speeds to the order of 1 to 2 Weston have been obtained. Further increases of development time beyond 24 minutes give washed out prints and unbalanced colors. Such a procedure would be carried out as follows:

1. First develop 24' at 68 F. in the following solution:

|                    | Grams |
|--------------------|-------|
| Metol              | 3     |
| Sodium sulfite     | 50    |
| Hydroquinone       | 6     |
| Sodium carbonate   | 40    |
| Sodium thiocyanate | 2     |
| Potassium bromide  | 2     |
| Water to make 1 l. |       |

## 6

2. Short stopped 3' after the first developer in  
Sodium bisulfite, 50 g.  
Water to make 1 l.

3. Wash for 2'.  
4. Second exposed 2'.  
5. Color developer 12' in the following developer:

|                             | Grams |
|-----------------------------|-------|
| P-amino diethyl aniline HCl | 4     |
| Sodium sulfite              | 20    |
| Sodium carbonate            | 80    |
| Hydroxylamine HCl           | 1     |
| Potassium bromide           | 2.5   |

6. Rinse 1'.  
7. Harden 5' in a solution of 3% potassium chrome alum.  
8. Wash for 10'.  
9. Bleach 10' in the following solution

|                        |       |
|------------------------|-------|
| Potassium ferricyanide | g 150 |
| Potassium bromide      | g 15  |
| Disodium phosphate     | g 40  |
| Sodium bisulfate       | g 25  |
| Formalin               | cc 20 |

Water to make 1 l.

10. Wash 5'.  
11. Fix 5' in the following solution:

|       | Grams |
|-------|-------|
| Hypo  | 200   |
| Borax | 5     |

Water to make 1 l.

12. Wash 10'.  
13. Dry.

A camera exposure made directly on Ansco Color Printon using an exposure  $\frac{1}{5}$  second at f4.5 and processed as above gave satisfactory color prints.

40 However, it was determined that if .05 gram per liter of thallous sulfate were added to the first developer the required first developing time could be reduced to 12 minutes at 68 F. and would give a satisfactory development as compared to 24 minutes without the thallous salt. Furthermore, the emulsion speed thus obtained with the thallous salt is three times as much as that of the plain developer, the gradation is made more brilliant and pleasing, and the color balance is not disturbed as much as by increased development time with the plain developer.

I claim:

1. A photographic developer solution for the initial development of an exposed color reversal photographic element having at least one silver halide emulsion layer containing color formers which will couple with the oxidation product of a p-phenylene diamine developing agent to form the dye image which comprises metol, hydroquinone, and a soluble thallium salt, the latter being in the proportion of 0.01 to 0.1 gram of the thallium salt per liter of solution, said developer solution being incapable of reacting with the color formers.

2. The photographic developer solution of claim 1 wherein the soluble thallium salt is thallium nitrate.

3. A photographic developer solution for the initial development of a reversal color photographic element having at least one silver halide emulsion layer containing color formers which will couple with the oxidation product of a p-phenylene diamine developing agent to form the dye image which comprises metol, hydroquinone,

7  
sodium sulfate, sodium carbonate, sodium thiocyanate, and from 0.01 to 0.1 gram of thallium nitrate per liter of solution, said developer solution being incapable of reacting with the color formers.

JAMES E. BATES.

REFERENCES CITED

The following references are of record in the file of this patent:

UNITED STATES PATENTS

|           |        |               |
|-----------|--------|---------------|
| Number    | Name   | Date          |
| 2,053,525 | Kieser | Sept. 8, 1936 |

8  
Number Name Date  
2,073,621 Blaney Mar. 16, 1937  
2,105,274 Steigmann Jan. 11, 1938

FOREIGN PATENTS

|          |               |              |
|----------|---------------|--------------|
| 5 Number | Country       | Date         |
| 477,628  | Great Britain | Jan. 4, 1938 |

OTHER REFERENCES

|    |                                                                                            |
|----|--------------------------------------------------------------------------------------------|
| 10 | Haidrich, <i>Photographische Korrespondenz</i> ,<br>Band 73, 1937, pp. 129-134, all cited. |
|    | Haidrich, <i>Photographische Korrespondenz</i> ,<br>Band 74, 1938, pp. 8-13, all cited.    |